# EUROPEAN PATENT SPECIFICATION

(11) **EP 2 572 891 B1**
(45) Date of publication and mention of the grant of the patent: **02.03.2016**
(21) Application number: 10850475.4
(22) Date of filing: 27.04.2010
(51) Int. Cl.: B41N 3/00, B41N 1/04, G03F 7/09, B41C 1/10, B41N 1/00, B41N 1/08

(54) **PLATE MATERIAL FOR DIRECT PLATEMAKING OF INK-JET PRINTING AND INK-JET PRINTING METHOD**
PLATTENMATERIAL FÜR DIREKTE PLATTENHERSTELLUNG FÜR TINTENSTRAHLDRUCK UND TINTENSTRAHLDRUCKVERFAHREN
MATÉRIAU DE CLICHÉ POUR FABRICATION DE CLICHÉ DIRECTE D'IMPRESSION À JET D'ENCRE ET PROCÉDÉ D'IMPRESSION À JET D'ENCRE

(43) Date of publication of application: 27.03.2013
(73) Proprietor: Institute Of Chemistry, Chinese Academy Of Sciences, Beijing 100190 (CN)
(72) Inventor: ZHOU, Haihua, Beijing 100190 (CN); SONG, Yanlin, Beijing 100190 (CN)
(74) Representative: Nederlandsch Octrooibureau
(86) International application number: PCT/CN2010/072239
(87) International publication number: WO 2011/134142

(56) References cited:
- CN-A- 1 315 483
- CN-A- 1 799 859
- CN-A- 101 397 438
- CN-A- 101 422 992
- JP-A- 2004 358 818
- US-A- 3 894 873
- US-A- 5 688 864
- US-B1- 6 187 380

## Description

### Field of the Invention

The present invention pertains to the field of printing plate, and particularly relates to a plate for inkjet computer-to-plate and an inkjet printing method.

### Background of the Invention

Offset lithographic printing is dominant in Chinese printing industry owing to its excellent performance. At present, the main printing substrate is aluminum substrate, and other metallic substrate, such as copper substrate and zinc substrate, can also be used. The aluminum substrate is generally undergoes treatments of anodizing and graining, so as to improve the printing durability and the resolution of aluminum plate (refer to CN85100875A). Through investigation, it is found that for a large-scale anodizing factory for aluminum substrate, the consumption of electric energy is 2,000,000 KWh per month, which leads to a cost of about $160,000/month, and in order to produce 10,000 m² of aluminum substrate, the output of the waste acid solution is about two tons and the output of the waste base solution is about three tons. The discharge of a large amount of the waste acid solution and the waste base solution has caused serious environmental pollution. Printing plates comprising an aluminum substrate are also known from US 3894873 and US 6187380 B.

### Summary of the Invention

An object of the present invention is to provide a plate for inkjet computer-to-plate with excellent printing durability and resolution, which can be obtained without the treatments of electrolytic graining and anodizing, so as to overcome the environmental hazard resulted from the waste acid solution and the waste base solution produced in the process of electrolytic graining and anodizing of metallic substrates in the prior art.

Another object of the present invention is to provide an inkjet printing method using the plate of the present invention.

According to the first object of the present invention, a plate for inkjet computer-to-plate is provided, which comprises a metallic base, an adhesive layer coated on the surface of the metallic base and an ink repulsive layer coated on the adhesive layer as defined in claim 1.

The adhesive in the adhesive layer is at least one selected from the group consisting of epoxy resin, polyurethane, polyolefin, polyester, styrene-butadiene rubber, gelatin, polyvinyl butyral, polyamide, rosin resin, polyvinyl alcohol, alkyd resin, polyvinyl acetate. The polyolefin is at least one selected from the group consisting of polypropylene, polyvinyl chloride and polystyrene.

The ink-repulsive layer is fluorine-containing resin.

The plate of the present invention can further comprise a protective layer, which is covered on the ink-repulsive layer. Preferably, the protective layer is a polymer film with a thickness of 1∼20 µm.

The polymer in the polymer film may be at least one selected from polyethylene, polypropylene, polypentene, polyvinylidene, polyallene, polyvinyl alcohol, polyvinyl butyral, polystyrene, polyethylene terephthalate, polyvinyl chloride, poly(vinylidene dichloride) resin and etc.

The adhesive layer is obtained by coating and drying adhesive sol. The adhesive sol for coating consists of solute and solvent. The concentration of the solute in the adhesive sol may be 0.05∼15 wt% and the coating amount of the adhesive sol may be 0.001∼10 g/m². Preferably, the adhesive layer is coated on the whole surface of the metallic base.

The solute in the adhesive sol is at least one selected from the group consisting of epoxy resin, polyurethane, polyolefin, polyester, styrene-butadiene rubber, gelatin, polyvinyl butyral, polyamide, rosin resin, polyvinyl alcohol, alkyd resin, polyvinyl acetate. The polyolefin is at least one selected from the group consisting of polypropylene, polyvinyl chloride and polystyrene.

The solvent in the adhesive sol may be at least one selected from the group consisting of water, ethanol, ester of diacid, cyclohexane, heptane, tetrahydrofuran and common aromatic solvents. The aromatic solvent is at least one selected from the group consisting of benzyl alcohol, phenethyl alcohol, xylol, ethylbenzene and toluene.

The ink-repulsive layer is obtained by coating an organic solution of fluorine-containing resin and drying. The content of fluorine-containing resin in the mixed liquid of fluorine-containing resin and organic solvent for coating may be 0.01∼20 wt% and the coating amount of the mixed liquid of fluorine-containing resin and organic solvent may be 0.001∼5 g/m². Preferably, the ink-repulsive layer is coated on the whole surface of the metallic base.

The fluorine-containing resin may be at least one selected from fluorine-containing acrylic resin, fluorine-containing isocyanate resin, fluorine-containing epoxy resin, fluorine-containing polyolefin resin and etc. The olefin in the fluorine-containing polyolefin resin is at least one selected from polypropylene, polyvinyl chloride, polystyrene and etc.

The organic solvent may be at least one selected from the group consisting of dimethyl sulfoxide, xylol, butyl acetate, ethylene glycol, propanediol, butanol, acetone, chloroform and etc.

The metallic base may be aluminum base used in ordinary printing production, or alloy base. The alloy base may be an alloy base of silica and aluminum. The content of silica in the alloy base is 30∼60 wt% (during smelting of aluminum, silica accounting for 30∼60 wt% of the total amount of silica and aluminum is added). An alloy base of aluminum and zinc, in which a content of the zinc is 1∼3 wt% or an alloy base of aluminum and iron, in which a content of the iron is 0.1∼1 wt% may also be used. Aluminum base or silica-containing aluminum alloy base is preferred. According to the plate provided by the present invention, the metallic base skips the treatments of electrolytic graining and anodizing, and does not undergo the treatments of electrolytic graining and anodizing to avoid the production of waste acid solution and waste base solution, which are harmful to the environment.

The method for preparing the plate for inkjet computer-to-plate of the present invention may comprise the following steps: adhesive sol consisting of solute and solvent is coated on the surface of the metallic base, and an adhesive layer is obtained after the solvent is removed by drying; an ink repulsive liquid, which is a mixed liquid of fluorine-containing resin and organic solvent, is coated on the adhesive layer; an ink repulsive layer, which is fluorine-containing resin, is obtained after the solvent is removed by drying; as a result, the plate for inkjet computer-to-plate is obtained.

The plate for inkjet computer-to-plate may be further covered with a protective layer, which may be a polymer film having a thickness of 1∼20 µm, to obtain a plate for inkjet computer-to-plate with a protective layer.

The composition and coating amount of the adhesive sol have been described hereinbefore, so they are omitted herein for the purpose of brief.

The composition and coating amount of the organic solution of fluorine-containing resin have been described hereinbefore, so they are omitted herein for the purpose of brief.

The metallic base used in the present invention without undergoing the treatments of electrolytic graining and anodizing is coated with adhesive on the surface and then coated with an ink-repulsive liquid, to obtain a plate for inkjet computer-to-plate. The obtained plate for inkjet computer-to-plate may be further covered with a polymer film as a protective layer, to protect the plate from scratch during transport. The coating adhesive on the surface of the metallic plate has an effect of enhancing the binding power between the metallic base and the ink-repulsive liquid. Due to low surface tension, the obtained ink-repulsive layer is not sticky to the printing ink during printing.

According to another object of the present invention, an inkjet printing method is provided, comprising the following steps: imparting image-text information on the plate of the present invention by using plate-making ink, and printing the plate having the image-text information, so as to obtain a presswork as defined in claim 9. The printing area with plate-making ink is an image-text zone, which shows affinity to ink during printing, while the area without plate-making ink is a non-image-text zone, which is not sticky to ink during printing, thereby realizing the contrast between the text-image zone and the non-text-image zone. By using the plate of the present invention, excellent printing durability and resolution can be obtained.

The method for printing image-text information on a plate with plate-making ink and the method for using the plate with image-text information to print may be conventional methods in the art.

If the plate has a protective layer, the film as the protective layer is removed before printing.

The plate-making ink may be various kinds of environment friendly water-based ink or solvent-based ink suitable for plate making.

Preferably, the plate-making ink is solvent-based ink, which comprises:

| | |
|---|---|
| film forming resin | 1∼35 wt% |
| curing agent | 0.01∼5 wt% |
| nano-scale or micron-scale dyestuff | 0.01∼10 wt% |
| solvent | balance amount. |

According to the preferred embodiment, the printing durability and resolution may be further improved.

The method for preparing the solvent-based plate-making ink may comprise the following steps: mixing 1∼35 wt% film forming resin, 0.01∼5 wt% curing agent, 0.01∼10 wt% nano-scale or micron-scale dyestuff and balance amount of solvent, stirring the mixed solution at room temperature till the solid solute is thoroughly dissolved, and filtering the obtained solution to remove the undissolved particles and impurities, and the obtained filtrate is solvent-based plate-making ink of the present invention.

The film forming resin in the plate-making ink is at least one selected from the group consisting of polyacrylic acid resin, polymethacrylic acid resin, ester of polyacrylic acid resin, ester of polymethacrylic acid resin, polyimide resin, methyl silicone resin, polyester resin, epoxy resin, phenolic resin, polyurethane resin, benzoxazine resin, alkyd resin, rubber, polyamide, polyvinyl chloride, polystyrene, polycarbonate, polyphenyl ether, polysulfone and etc.

The ester of polyacrylic acid resin comprises a product of esterification reaction between the polyacrylic acid resin and C1∼C5 monobasic alcohols. When the reactants are added, the molar ratio between polyacrylic acid resin and monobasic alcohols may be 1 : 10∼10 : 1. The ester of the polymethacrylic acid resin comprises a product of esterification reaction between the polymethacrylic acid resin and C1∼C5 monobasic alcohols. When the reactants are added, the molar ratio between polymethacrylic acid resin and monobasic alcohols may be 1 : 10∼10 : 1.

The curing agent in the plate-making ink may be at least one selected from the group consisting of silicone oil, epoxy resin with a low molecular weight, dicyandiamide, melamine, ethanolamine, triethylamine, polyisocyanate, benzoyl peroxide, acetic anhydride, 2-ethylimidazole, 2,4-dimethyl imidazole, mellophanic dianhydride and N,N-dimethylaniline.

The epoxy equivalent value of the epoxy resin with a low molecular weight may be 100∼2000 g/equivalent.

The particle size of the nano-scale or micron-scale dyestuff in the plate-making ink may be 10∼3000 nm.

The dyestuff in the plate-making ink may be one of acidic dyestuff, active dyestuff or alkaline dyestuff.

The acidic dyestuff may be one of dye acid blue 9, dye acid blue 9 SF and dye acid yellow 23 SF. The active dyestuff may be one of black dyestuff SP series or reactive black. The alkaline dyestuff may be one of basic brilliant blue and N,N-dimethylaniline in blue dyestuff.

The solvent in the plate-making ink may be one selected from ethylene glycol monomethyl ether, ethylene glycol monoethyl ether, ethylene glycol mono-*n*-butyl ether, ethylene glycol dimethyl ether, propylene glycol monomethyl ether, propylene glycol monoethyl ether, propylene glycol monomethyl ether acetate, propylene glycol monoethyl ether acetate, propylene glycol monobutyl ether acetate, ethylene glycol monobutyl ether acetate, N,N-dimethylformamide, dioxane, sec-butyl acetate, A grade mineral essential oil and B grade mineral essential oil.

The plate for inkjet computer-to-plate of the present invention can achieve excellent printing durability and resolution without making the metallic base undergo the treatments of electrolytic graining and anodizing, thereby avoiding the serious environmental hazard of waste acid solution and waste base solution produced in the process of electrolytic graining and anodizing.

### Detailed Description of the Embodiments

In the following a reference example is not an embodiment of the present invention but represents background art or is useful for understanding the invention.

### Example 1 (reference example)

After an industrial aluminum base without undergoing the treatments of electrolytic graining and anodizing is degreased with a dilute aqueous solution of sodium hydroxide at a concentration of 5 wt% and washed with water, adhesive sol is coated on the surface of the aluminum base by method of spin coating. The coated adhesive sol is a benzyl alcohol solution of epoxy resin at a concentration of 0.05 wt%. The coating amount of the adhesive sol is 0.001 g/m². Benzyl alcohol is removed by drying, to obtain an epoxy resin adhesive. An ink repulsive liquid consisting of polydimethylsiloxane and silicone oil is coated on the adhesive layer of epoxy resin. The mass ratio between polydimethylsiloxane and silicone oil is 5 : 1. The coating amount of the ink repulsive liquid is 5 g/m². Polydimethylsiloxane is cured by drying to obtain an ink repulsive layer, which is formed from a mixture of polydimethylsiloxane and silicone oil. Thereby, an aluminum plate for inkjet computer-to-plate is obtained. A polyethylene film with a thickness of 1 µm is covered on the obtained aluminum plate as the protective film.

1 wt% polyacrylic acid resin, 5 wt% triethanolamine, 0.01 wt% basic brilliant blue (with a particle size of 10 nm) and the balance amount of ethylene glycol dimethyl ether, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 2 (reference example)

After an industrial aluminum alloy base (containing SiO₂ at a content of 60 wt%) without electrolytic graining and anodizing is degreased with a dilute aqueous solution of sodium hydroxide at a concentration of 5 wt% and washed with water, adhesive sol is coated on the surface of the aluminum base by method of spin coating. The coated adhesive sol is a benzyl alcohol solution of epoxy resin at a concentration of 15 wt%. The coating amount of the adhesive sol is 10 g/m². Benzyl alcohol is removed by drying, to obtain an adhesive layer of epoxy resin. An ink repulsive liquid consisting of polymethylvinylsiloxane and methyl silicone oil is coated on the adhesive layer of epoxy resin. The mass ratio between polymethylvinylsiloxane and methyl silicone oil is 15 : 1. The coating amount of the ink repulsive liquid is 0.001 g/m². Polymethylvinylsiloxane is cured by drying to obtain an ink repulsive layer, which is formed from a mixture of polymethylvinylsiloxane and methyl silicone oil. Thereby, an aluminum plate for inkjet computer-to-plate is obtained. A polypropene film with a thickness of 20 µm is covered on the obtained aluminum plate as the protective film.

35 wt% phenolic resin, 0.01 wt% epoxy resin with an epoxy equivalent value of 100 g/equivalent, 0.01 wt% black dyestuff SP (with a particle size of 3000 nm) and the balance amount of ethylene glycol mono-methyl ether, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 3 (embodiment of the invention)

After an industrial aluminum base without electrolytic graining and anodizing is degreased with a dilute aqueous solution of sodium hydroxide at a concentration of 5 wt% and washed with water, adhesive sol is coated on the surface of the aluminum base by method of spin coating. The coated adhesive sol is a xylene solution of polyurethane at a concentration of 0.05 wt%. The coating amount of the adhesive sol is 1 g/m². The xylene is removed by drying, to obtain an adhesive layer of polyurethane. An ink repulsive liquid consisting of dimethylsulfoxide solution of fluorine-containing isocyanate resin at a concentration of 20 wt% is coated on the adhesive layer of polyurethane resin. The coating amount of the ink repulsive liquid is 5 g/m². Dimethylsulfoxide is removed by drying to obtain an ink repulsive layer, which is formed from fluorine-containing isocyanate resin. Thereby, an aluminum plate for inkjet computer-to-plate is obtained. A polypentene film with a thickness of 10 µm is covered on the obtained aluminum plate as the protective film.

20 wt% epoxy resin, 2 wt% polyisocyanate, 10 wt% dye acid blue 9 (with a particle size of 2000 nm) and the balance amount of ethylene glycol mono-*n*-butyl ether, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 4 (invention)

After an industrial aluminum alloy base (containing SiO₂ at a content of 40 wt%) without undergoing the treatments of electrolytic graining and anodizing is degreased with a 5 wt% dilute aqueous solution of sodium hydroxide at a concentration of 5 wt% and washed with water, adhesive sol is coated on the surface of the aluminum alloy base by method of spin coating. The coated adhesive sol is xylol solution of polyurethane at a concentration of 15 wt%. The coating amount of the adhesive sol is 2 g/m². Xylol is removed by drying to obtain a polyurethane adhesive layer. An ink repulsive liquid consisting of xylol solution of fluorine-containing acrylic resin at a concentration of 0.01 wt% is coated on the polyurethane adhesive layer. The coating amount of the ink repulsive liquid is 0.001 g/m². Xylol is removed by drying to obtain an ink repulsive layer, which is formed from fluorine-containing acrylic resin. Thereby, aluminum plate for inkjet computer-to-plate is obtained. A polyvinylidene film with a thickness of 10 µm is covered on the obtained aluminum plate as the protective layer.

15 wt% polyimide resin, 0.03 wt% triethylamine, 5 wt% reactive black (with a particle size of 30 nm) and the balance amount of propylene glycol mono-methyl ether acetate, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 5 (reference example)

After an industrial aluminum alloy base (containing SiO₂ at a content of 30 wt%) without undergoing the treatments of electrolytic graining and anodizing is degreased with a dilute aqueous solution of sodium hydroxide at a concentration of 5 wt% and washed with water, adhesive sol is coated on the surface of the aluminum base by method of spin coating. The coated adhesive sol is tetrahydrofuran solution of polystyrene at a concentration of 0.05 wt%. The coating amount of the adhesive sol is 1.5 g/m². Tetrahydrofuran is removed by drying to obtain a polystyrene adhesive layer. An ink repulsive liquid consisting of polyphenylmethylsiloxane and dibutyltin dilaurate is coated on the polystyrene adhesive layer. The mass ratio between polyphenylmethylsiloxane and dibutyltin dilaurate is 6 : 1. The coating amount of the ink repulsive liquid is 2 g/m². Polyphenylinethylsiloxane is cured by drying to obtain an ink repulsive layer, which is formed from a mixture of polyphenylmethylsiloxane and dibutyltin dilaurate. Thereby, an aluminum plate for inkjet computer-to-plate is obtained. A polyallene with a thickness of 5 µm is covered on the obtained aluminum plate as the protective layer.

35 wt% polymethacrylic acid resin, 4 wt% melamine, 1 wt% N,N-dimethylaniline (with a particle size of 100 nm) and the balance amount of ethylene glycol monoethyl ether, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 6 (reference example)

After an industrial aluminum alloy base (containing SiO₂ at a content of 60 wt%) without undergoing the treatments of electrolytic graining and anodizing is degreased with a dilute aqueous solution of sodium hydroxide at a concentration of 5 wt% and washed with water, the aluminum alloy base is subject to coat by method of spin coating. Adhesive sol is coated on the surface of the aluminum alloy base. The coated adhesive sol is a benzyl alcohol solution of polystyrene at a concentration of 15 wt%. The coating amount of the adhesive sol is 2.5 g/m². Benzyl alcohol is removed by drying to obtain a polystyrene adhesive layer. An ink repulsive liquid consisting of polymethylethylsiloxane and aminosilane is coated on the polystyrene adhesive layer. The mass ratio between polymethylethylsiloxane and aminosilane is 8 : 1. The coating amount of the ink repulsive liquid is 1 g/m². Polymethylethylsiloxane is cured by drying to obtain an ink repulsive layer, which is formed from a mixture of polymethylethylsiloxane and aminosilane. Thereby, an aluminum plate for inkjet computer-to-plate is obtained. A polyvinyl alcohol film with a thickness of 12 µm is covered on the obtained aluminum plate as a protective layer.

5 wt% methyl silicone resin, 0.03 wt% dicyandiamide, 0.01 wt% silicone oil, 1 wt% dye acid yellow 23 SF (with a particle size of 1000 nm) and the balance amount of propylene glycol monomethyl ether, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 7 (invention)

After an industrial aluminum alloy base (containing SiO₂ at a content of 40 wt%) without undergoing the treatments of electrolytic graining and anodizing is degreased with a dilute aqueous solution of sodium hydroxide at a concentration of 5 wt% and washed with water, the aluminum alloy base is subject to coat by method of spin coating. Adhesive sol is coated on the surface of the aluminum alloy base. The coated adhesive sol is an aqueous solution of gelatin at a concentration of 0.05 wt%. The coating amount of the adhesive sol is 4 g/m². Water is removed by drying to obtain a gelatin adhesive layer. An ink repulsive liquid consisting of a butyl acetate solution of fluorine-containing epoxy resin at a concentration of 0.01 wt% is coated on the gelatin adhesive layer. The coating amount of the ink repulsive liquid is 0.005 g/m². Butyl acetate is removed by drying to obtain an ink repulsive layer, which is formed from fluorine-containing epoxy resin. Thereby, an aluminum plate for inkjet computer-to-plate is obtained. A polyvinyl butyral film with a thickness of 6µm is covered on the obtained aluminum plate as a protective layer.

5 wt% product of the reaction between polyacrylic acid resin and methanol (during addition of reactants, the molar ratio between polyacrylic acid and methanol is 1 : 2), 0.03 wt% epoxy resin with an epoxy equivalent value of 2000 g/equivalent, 1 wt% basic brilliant blue (with a particle size of 2000 nm) and the balance amount of propylene glycol monoethyl ether, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 8 (invention)

After an industrial aluminum alloy base (containing SiO₂ at a content of 50 wt%) without undergoing the treatments of electrolytic graining and anodizing is degreased with a dilute aqueous water solution of sodium hydroxide at a concentration of 5 wt% and washed with water, the aluminum alloy base is subject to coat by method of spin coating. Adhesive sol is coated on the surface of the aluminum base. The coated adhesive sol is an aqueous solution of gelatin at a content of 15 wt%. The coating amount of the adhesive sol is 1.5 g/m². Water is removed by drying to obtain a gelatin adhesive layer. An ink repulsive liquid consisting of ethylene glycol (40 wt%) and propanediol (40 wt%) solution of fluorine-containing polyethylene resin at a concentration of 20 wt% is coated on the gelatin adhesive layer. The coating amount of the ink repulsive liquid is 3 g/m². Ethylene glycol and propanediol are removed by drying to obtain an ink repulsive layer, which is formed from fluorine-containing polyethylene resin. Thereby, an aluminum plate for inkjet computer-to-plate is obtained. A polystyrene film with a thickness of 3µm is covered on the obtained aluminum plate as a protective layer.

5 wt% product of the reaction between polymethacrylic acid resin and methanol (during addition of reactants, the molar ratio between polymethacrylic acid and methanol is 1 : 2), 0.03 wt% epoxy resin with an epoxy equivalent value of 100g/equivalent, 1 wt% basic brilliant blue (with a particle size of 2000 nm) and the balance amount of propylene glycol monoethyl ether acetate, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 9 (reference example)

After an industrial aluminum alloy base (containing SiO₂ at a content of 30 wt%) without undergoing treatments of electrolytic graining and anodizing is degreased with a dilute aqueous solution of sodium hydroxide at a content of 5 wt% and washed with water, the aluminum alloy base is subject to coat by method of spin coating. Adhesive sol is coated on the surface of the aluminum alloy plate. The coated adhesive sol is an ethanol solution of alkyd resin at a concentration of 0.05 wt%. The coating amount of the adhesive sol is 0.5 g/m². Ethanol is removed by drying to obtain an alkyd resin adhesive layer. An ink repulsive liquid consisting of polymethylpropylsiloxane and aminopropyl silane is coated on the alkyd resin adhesive layer. The mass ratio between polymethylpropylsiloxane and aminopropyl silane is 10 : 1. The coating amount of the ink repulsive liquid is 0.01 g/m². Polymethylpropylsiloxane is cured by drying to obtain an ink repulsive layer, which is formed from a mixture of polymethylpropylsiloxane and aminopropyl silane. Thereby, an aluminum plate for inkjet computer-to-plate is obtained. A polyethylene terephthalate film with a thickness of 16 µm is covered on the obtained aluminum plate as the protective layer.

20 wt% polyester resin, 0.02 wt% benzoyl peroxide, 0.02 wt% black dyestuff SP (with a particle size of 3000 nm) and the balance amount of propylene glycol monobutyl ether acetate, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 10 (reference example)

After an industrial aluminum alloy base (containing SiO₂ at a content of 30 wt%) without undergoing the treatments of electrolytic graining and anodizing is degreased with a dilute aqueous solution of sodium hydroxide at a concentration of 5 wt% and washed with water, the aluminum alloy base is subject to coat by method of spin coating. Adhesive sol is coated on the surface of the aluminum alloy base. The coated adhesive sol is an ethanol solution alkyd resin at a concentration of 15 wt%. The coating amount of the adhesive sol is 0.02 g/m². Ethanol is removed by drying to obtain an alkyd resin adhesive layer. An ink repulsive liquid consisting of polymethylcyclohexylsiloxane and dibutyltin dilaurate is coated on the alkyd resin adhesive layer. The mass ratio between polymethylcyclohexylsiloxane and dibutyltin dilaurate is 12 : 1. The coating amount of the ink repulsive liquid is 0.005 g/m². Polymethylcyclohexylsiloxane is cured by drying to obtain an ink repulsive layer, which is formed from a mixture of polymethylcyclohexylsiloxane and dibutyltin dilaurate. Thereby, an aluminum plate for inkjet computer-to-plate is obtained. A polyvinyl chloride film with a thickness of 9 µm is covered on the obtained aluminum plate as the protective layer.

20 wt% rubber, 0.02 wt% benzoyl peroxide, 0.02 wt% black dyestuff SP (with a particle size of 3000 nm) and the balance amount of ethyl glycol monobutyl ether acetate, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 11 (invention)

After an industrial aluminum base without undergoing the treatments of electrolytic graining and anodizing is degreased with a dilute aqueous solution of sodium hydroxide at a concentration of 5 wt% and washed with water, the aluminum alloy base is subject to coat by method of spin coating. Adhesive sol is coated on the surface of the aluminum base. The coated adhesive sol is ester of diacid solution of polyester at a concentration of 0.05 wt%. The coating amount of the adhesive sol is 0.005 g/m². Ester of diacid is removed by drying to obtain a polyester adhesive layer. An ink repulsive liquid consisting of a butanol solution of fluorine-containing acrylic resin at a content of 0.01 wt% is coated on the polyester adhesive layer. The coating amount of the ink repulsive liquid is 4 g/m². Butanol is removed by drying to obtain an ink repulsive layer, which is formed from fluorine-containing acrylic resin. Thereby, an aluminum plate for inkjet computer-to-plate is obtained. A poly(vinylidene dichloride) film with a thickness of 8 µm is covered on the obtained aluminum plate as the protective layer.

1 wt% polystyrene, 4 wt% N,N-dimethylaniline, 10 wt% acid blue 9 (with a particle size of 800 nm) and the balance amount of N,N-dimethylformamide, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 12 (invention)

After an industrial aluminum alloy base (containing SiO₂ at a content of 40 wt%) without undergoing the treatments of electrolytic graining and anodizing is degreased with a dilute aqueous solution of sodium hydroxide at a concentration of 5 wt% and washed with water, the aluminum alloy base is subject to coat by method of spin coating. Adhesive sol is coated on the surface of the aluminum alloy base. The coated adhesive sol is an ester of diacid solution of polyester at a concentration of 15 wt%. The coating amount of the adhesive sol is 0.01 g/m². Ester of diacid is removed by drying to obtain a polyester adhesive layer. An ink repulsive liquid consisting of an acetone solution of fluorine-containing epoxy resin at a concentration of 20 wt% is coated on the polyester adhesive layer. The coating amount of the ink repulsive liquid is 0.2 g/m². Acetone is removed by drying to obtain an ink repulsive layer, which is formed from fluorine-containing epoxy resin. Thereby, an aluminum plate for inkjet computer-to-plate is obtained. A polyethylene terephthalate film with a thickness of 2 µm is covered on the obtained aluminum plate as the protective layer.

1 wt% polyamide, 4 wt% N,N-dimethylaniline, 10 wt% acid blue 9 (with a particle size of 800 nm) and the balance amount of dioxane, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 13 (reference example)

After an industrial aluminum alloy base (containing SiO₂ at a content of 45 wt%) without undergoing the treatments of electrolytic graining and anodizing is degreased with a dilute aqueous solution of sodium hydroxide at a concentration of 5 wt% and washed with water, the aluminum alloy base is subject to coat by method of spin coating. Adhesive sol is coated on the surface of the aluminum base. The coated adhesive sol is an aqueous solution of polyvinyl alcohol at a concentration of 0.05 wt%. The coating amount of the adhesive sol is 0.06 g/m². Water is removed by drying to obtain a polyvinyl alcohol adhesive layer. An ink repulsive liquid consisting of polymethylisobutylsiloxane and methoxy silane is coated on the polyvinyl alcohol adhesive layer. The mass ratio between polymethylisobutylsiloxane and methoxy silane is 9 : 1. The coating amount of the ink repulsive liquid is 2.5 g/m². Polymethylisobutylsiloxane is cured by drying to obtain an ink repulsive layer, which is formed from a mixture of polymethylisobutylsiloxane and methoxy silane. Thereby, an aluminum plate for inkjet computer-to-plate is obtained. A polypentylene film with a thickness of 13 µm is covered on the obtained aluminum plate as the protective layer.

35 wt% product of the reaction between polyacrylic acid resin and pentanol (during addition of reactants, the molar ratio between polyacrylic acid resin and pentanol is 1 : 2), 0.02 wt% diethanolamine, 1 wt% dye acid yellow 23 SF (with a particle size of 2000 nm) and the balance amount of *sec*-butyl acetate, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 14 (reference example)

After an industrial aluminum alloy base (containing SiO₂ at a content of 35 wt%) without undergoing the treatments of electrolytic graining and anodizing is degreased with a dilute aqueous solution of sodium hydroxide at a concentration of 5 wt% and washed with water, the aluminum alloy base is subject to coat by method of spin coating. Adhesive sol is coated on the surface of the aluminum alloy plate. The coated adhesive sol is an aqueous solution of polyvinyl alcohol at a concentration of 15 wt%. The coating amount of the adhesive sol is 0.45 g/m². Water is removed by drying to obtain a polyvinyl alcohol adhesive layer. An ink repulsive liquid consisting of polyethylvinylsiloxane and ethyoxyl silane is coated on the polyvinyl alcohol adhesive layer. The mass ratio between polyethylvinylsiloxane and ethyoxyl silane is 7 : 1. The coating amount of the ink repulsive liquid is 1.5 g/m². Polyethylvinylsiloxane is cured by drying to obtain an ink repulsive layer, which is formed from a mixture of polyethylvinylsiloxane and ethyoxyl silane. Thereby, an aluminum plate for inkjet computer-to-plate is obtained. A polyallene film with a thickness of 1µm is covered on the obtained aluminum plate as the protective layer.

35 wt% polyvinyl chloride, 0.02 wt% diethanolamine, 1 wt% dye acid yellow 23 SF (with a particle size of 2000 nm) and the balance amount of A grade mineral essential oil, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 15 (invention)

After an industrial aluminum alloy base (containing SiO₂ at a content of 60 wt%) without undergoing the treatments of electrolytic graining and anodizing is degreased with a dilute aqueous solution of sodium hydroxide at a concentration of 5 wt% and washed with water, the aluminum alloy base is subject to coat by method of spin coating. Adhesive sol is coated on the surface of the aluminum alloy plate. The coated adhesive sol is an ethylbenzene solution of polyvinyl acetate at a concentration of 0.05%. The coating amount of the adhesive sol is 0.004 g/m². Ethylbenzene is removed by drying to obtain a polyvinyl acetate adhesive layer. An ink repulsive liquid consisting of a chloroform solution of fluorine-containing isocyanate at a concentration of 20 wt% is coated on the polyvinyl acetate adhesive layer. The coating amount of the ink repulsive liquid is 0.5 g/m². Chloroform is removed by drying to obtain an ink repulsive layer, which is formed from fluorine-containing isocyanate. Thereby, an aluminum plate for inkjet computer-to-plate is obtained. A polystyrene film with a thickness of 10 µm is covered on the obtained aluminum plate as the protective layer.

20 wt% polycarbonate, 0.01 wt% N,N-dimethylaniline, 0.01 wt% black dyestuff SP (with a particle size of 3000 nm) and the balance amount of B grade mineral essential oil, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 16 (invention)

After an industrial aluminum alloy base (containing SiO₂ at a content of 30 wt%) without undergoing the treatments of electrolytic graining and anodizing is degreased with a dilute aqueous solution of sodium hydroxide at a concentration of 5 wt% and washed with water, the aluminum alloy base is subject to coat by method of spin coating. Adhesive sol is coated on the surface of the aluminum base. The coated adhesive sol is an ethylbenzene solution of polyvinyl acetate at a concentration of 15%. The coating amount of the adhesive sol is 9 g/m². Ethylbenzene is removed by drying to obtain a polyvinyl acetate adhesive layer. An ink repulsive liquid consisting of a dimethylsulfoxide solution of fluorine-containing polyethylene at a concentration of 0.01 wt% is coated on the polyvinyl acetate adhesive layer. The coating amount of the ink repulsive liquid is 3 g/m². Dimethylsulfoxide is removed by drying to obtain an ink repulsive layer, which is formed from fluorine-containing polyethylene. Thereby, an aluminum plate for inkjet computer-to-plate is obtained. A polyvinyl butyral film with a thickness of 5µm is covered on the obtained aluminum plate as the protective layer.

1 wt% polyphenyl ether, 0.01 wt% N,N-dimethylaniline, 0.01 wt% black dyestuff SP (with a particle size of 3000 nm) and the balance amount of ethylene glycol monomethyl ether, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 17 (reference example)

After an industrial aluminum alloy base (containing SiO₂ at a content of 32 wt%) without undergoing the treatments of electrolytic graining and anodizing is degreased with a dilute aqueous solution of sodium hydroxide at a concentration of 5 wt% and washed with water, adhesive sol is coated on the surface of the aluminum alloy plate by method of spin coating. The coated adhesive sol is a benzyl alcohol solution of polyvinyl butyral at a concentration of 0.9 wt%. The coating amount of the adhesive sol is 0.015 g/m². Benzyl alcohol is removed by drying to obtain a polyvinyl butyral adhesive layer. An ink repulsive liquid consisting of polydimethylsiloxane and silicone oil is coated on the polyvinyl butyral adhesive layer. The mass ratio between polydimethylsiloxane and silicone oil is 7 : 1. The coating amount of the ink repulsive liquid is 5 g/m². Polydimethylsiloxane is cured by drying to obtain an ink repulsive layer, which is formed from a mixture of polydimethylsiloxane and silicone oil. Thereby, an aluminum plate for inkjet computer-to-plate is obtained. A polyethylene film with a thickness of 1 µm is covered on the obtained aluminum plate as the protective layer.

5 wt% polyurethane resin, 5 wt% triethanolamine, 0.01 wt% basic brilliant blue (with a particle size of 10 nm) and the balance amount of ethylene glycol dimethyl ether, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 18 (reference example)

After an industrial aluminum alloy base (containing SiO₂ at a content of 50 wt%) without undergoing the treatments of electrolytic graining and anodizing is degreased with a dilute aqueous solution of sodium hydroxide at a concentration of 5 wt% and washed with water, adhesive sol is coated on the surface of the aluminum alloy base by method of spin coating. The coated adhesive sol is a xylol solution of polyamide at a concentration of 10 wt%. The coating amount of the adhesive sol is 6 g/m². Xylol is removed by drying to obtain a polyamide adhesive layer. An ink repulsive liquid consisting of polymethylvinylsiloxane and methyl silicone oil is coated on the polyamide adhesive layer. The mass ratio between polymethylvinylsiloxane and methyl silicone oil is 8 : 1. The coating amount of the ink repulsive liquid is 0.001 g/m². Polymethylvinylsiloxane is cured by drying to obtain an ink repulsive layer, which is formed from a mixture of polymethylvinylsiloxane and silicone oil. Thereby, an aluminum plate for inkjet computer-to-plate is obtained. A polypropylene film with a thickness of 20 µm is covered on the obtained aluminum plate as the protective layer.

20 wt% alkyd resin, 0.01 wt% epoxy resin with an epoxy equivalent value of 100 g/equivalent, 0.01wt% black dyestuff SP (with a particle size of 3000 nm) and the balance amount of ethylene glycol monomethyl ether, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 19 (invention)

After an industrial aluminum alloy base (containing SiO₂ at a content of 45 wt%) without undergoing the treatments of electrolytic graining and anodizing is degreased with a dilute aqueous solution of sodium hydroxide at a concentration of 5 wt% and washed with water, adhesive sol is coated on the surface of the aluminum alloy plate by method of spin coating. The coated adhesive sol is a cyclohexane solution of rosin resin at a concentration of 1.5 wt%. The coating amount of the adhesive sol is 1.2 g/m². Cyclohexane is removed by drying to obtain a rosin resin adhesive layer. An ink repulsive liquid consisting of a dimethylsulfoxide solution of fluorine-containing isocyanate resin at a concentration of 20 wt% is coated on the rosin resin adhesive layer. The coating amount of the ink repulsive liquid is 5 g/m². Dimethylsulfoxide is removed by drying to obtain an ink repulsive layer, which is formed from fluorine-containing isocyanate resin. Thereby, an aluminum plate for inkjet computer-to-plate is obtained. A polypentylene film with a thickness of 10 µm is covered on the obtained aluminum plate as the protective layer.

15 wt% benzoxazine resin, 2 wt% polyisocyanate, 10 wt% dye acid blue 9 (with a particle size of 2000 nm) and the balance amount of ethylene glycol mono-*n*-butyl ether, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

### Example 20 (reference example)

After an industrial aluminum alloy base (containing SiO₂ at a content of 40 wt%) without undergoing the treatments of electrolytic graining and anodizing is degreased with a dilute aqueous solution of sodium hydroxide at a concentration of 5 wt% and washed with water, the aluminum alloy base is subject to coat by method of spin coating. Adhesive sol is coated on the surface of the aluminum alloy base. The coated adhesive sol is a heptane solution of styrene-butadiene rubber at a concentration of 3 wt%. The coating amount of the adhesive sol is 0.04 g/m². Heptane is removed by drying to obtain a styrene-butadiene rubber adhesive layer. An ink repulsive liquid consisting of polymethylcyclohexylsiloxane and dibutyltin dilaurate is coated on the styrene-butadiene rubber adhesive layer. The mass ratio between polymethylcyclohexylsiloxane and dibutyltin dilaurate is 10 : 1. The coating amount of the ink repulsive liquid is 0.01 g/m². Polymethylcyclohexylsiloxane is cured by drying to obtain an ink repulsive layer, which is formed from a mixture of polymethylcyclohexylsiloxane and dibutyltin dilaurate. Thereby, an aluminum plate for inkjet computer-to-plate is obtained. A polyvinyl chloride with a thickness of 9 µm is covered on the obtained aluminum plate as the protective layer.

15 wt% polysulfone, 5 wt% epoxy resin with an epoxy equivalent value of 100 g/equivalent, 0.01 wt% black dyestuff SP (with a particle size of 3000 nm) and the balance amount of ethylene glycol monomethyl ether, which constitute solvent-based plate-making ink, are mixed and stirred at room temperature till all solid solutes are thoroughly dissolved. The undissolved particles and impurities are removed by filtration. The obtained filtrate is the solvent-based plate-making ink.

The solvent-based plate-making ink obtained in Examples 1∼20 is respectively sprayed by an inkjet printer onto the aluminum plates for the inkjet computer-to-plate obtained in the corresponding example (removing the protective layer) to form images. Then the aluminum plates sprayed with the plate-making ink are baked at 90∼300 °C so that the plate-making ink is crosslinked to cure under the action of the curing agent in the plate-making ink. After the foregoing treatment, the aluminum plates are used to print on a machine. According to the test result, the printing plates have good printing suitability and the printing durability may reach about 100000 pieces. The resolution of the line in the image-text of the plates may reach 10 µm. 5∼95% of the dots are complete and clear.

### Example 21

Blackjet ink (SPECTRA, UK) is respectively sprayed by an inkjet printer onto the aluminum plates for inkjet computer-to-plate obtained in Examples 1-20 (removing the protective layer) to form images. Then the aluminum plates sprayed with the plate-making ink are baked at 90∼300 °C so that the plate-making ink is crosslinked to cure under the action of the curing agent in the plate-making ink. After the foregoing treatment, the aluminum plates are used to print on a machine. According to the test result, the printing plates have good printing suitability and the printing durability may reach about 10000 pieces. The resolution of the line in the image-text of the plates may reach 20 µm. 10∼90% of the dots are complete and clear.

### Example 22

Seiko ink (SOLVENT INK, Japan) is respectively sprayed by an inkjet printer onto the aluminum plates for inkjet computer-to-plate obtained in Examples 1-20 (removing the protective layer) to form images. Then the aluminum plates sprayed with the plate-making ink are baked at 90∼300 °C so that the plate-making ink is crosslinked to cured under the action of the curing agent in the plate-making ink. After the foregoing treatment, the aluminum plates are used to print on a machine. According to the result of the test, the printing plates have good printing suitability and the printing durability may reach about 50000 pieces. The resolution of the line in the image-text of the plates may reach 15 µm. 5-90% of the dots are complete and clear.

### Comparison Example 1

The industrial aluminum alloy base (containing SiO₂ at a content of 40 wt%) treated by electrolytic graining and anodizing (electrolyzed in a 1% HCl aqueous solution twice, 30s each time; anodized in a 15% H₂SO₄ aqueous solution) is degreased with a dilute aqueous solution of sodium hydroxide at a concentration of 5 wt% and washed with water, ink (SPT510, China) is sprayed on it by an inkjet printer to form an image. Then the aluminum plate sprayed with the plate-making ink is baked at 90∼300 °C so that the plate-making ink is crosslinked to cure under the action of the curing agent in the plate-making ink. After the foregoing treatment, the aluminum plate is used to print on a machine. According to the test result, the printing plate has good printing suitability and the printing durability may reach about 10000 pieces. The resolution of the lines in the image-text of the plate may reach 30 µm. 15∼85% of the dots are complete and clear.

### Comparison Example 2

After an industrial aluminum alloy base (containing SiO₂ at a content of 40 wt%) without undergoing the treatments of electrolytic graining and anodizing is degreased with a dilute aqueous solution of sodium hydroxide at a concentration of 5 wt% and washed with water, ink (P522-6, China) is sprayed on it by an inkjet printer to form an image. Then the aluminum plate sprayed with the plate-making ink is baked at 90∼300 °C so that the plate-making ink is crosslinked to cure under the action of the curing agent in the plate-making ink. After the foregoing treatment, the aluminum plate is used to print on a machine. According to the test result, the printing plate has good printing suitability and the printing durability may reach about 200 pieces. The resolution of the lines in the image-text of the plate only reaches 900 µm.

## Claims

1. A plate for inkjet computer-to-plate, comprising a metallic base, an adhesive layer coated on the surface of the metallic base and an ink repulsive layer coated on the adhesive layer, wherein the adhesive layer is obtained by coating and drying adhesive sol wherein the adhesive sol for coating consists of solute and solvent and wherein
the metallic base is without undergoing the treatments of electrolytic graining and anodizing,
adhesive in the adhesive layer is at least one selected from the group consisting of epoxy resin, polyurethane, polyolefin, polyester, styrene-butadiene rubber, gelatin, polyvinyl butyral, polyamide, rosin resin, polyvinyl alcohol, alkyd resin and polyvinyl acetate,
the ink repulsive layer is fluorine-containing resin.

2. The plate for inkjet computer-to-plate according to claim 1, **characterized in that** the ink repulsive layer is covered with a protective layer, which is a polymer film with a thickness of 1∼20 µm,
polymer in the polymer film is at least one of polyethylene, polypropylene, polypentene, polyvinyl alcohol, polyvinyl butyral, polystyrene, polyethylene terephthalate, polyvinyl chloride and poly(vinylidene dichloride).

3. The plate for inkjet computer-to-plate according to claim 1, **characterized in that** the concentration of the solute in the adhesive sol is 0.05∼15 wt%, and the coating amount of the adhesive sol is 0.001∼10 g/m², the solute is adhesive in the adhesive sol; and/or
the ink repulsive layer is obtained by coating a mixed liquid of fluorine-containing resin and organic solvent and drying, wherein the content of the fluorine-containing resin in the mixed liquid of fluorine-containing resin and organic solvent is 0.01∼20 wt%, and the coating amount of the mixed liquid of fluorine-containing resin and organic solvent is 0.001∼5 g/m².

4. The plate for inkjet computer-to-plate according to claim 1 or 3, **characterized in that** the polyolefin is at least one selected from the group consisting of polypropylene, polyvinyl chloride and polystyrene;
the fluorine-containing resin is at least one of fluorine-containing acrylic resin, fluorine-containing isocyanate resin, fluorine-containing epoxy resin and fluorine-containing polyolefin resin;
the organic solvent is at least one selected from the group consisting of dimethyl sulfoxide, xylol, butyl acetate, ethylene glycol, propanediol, butanol, acetone and chloroform.

5. The plate for inkjet computer-to-plate according to claim 3, **characterized in that** the solvent is at least one selected from the group consisting of water, ethanol, ester of diacid, cyclohexane, heptane, tetrahydrofuran and aromatic solvent.

6. The plate for inkjet computer-to-plate according to claim 5, **characterized in that** the aromatic solvent is at least one selected from the group consisting of benzyl alcohol, phenethyl alcohol, xylol, ethylbenzene and toluene.

7. The plate for inkjet computer-to-plate according to claim 1, **characterized in that** the metal base is aluminum base or alloy base.

8. The plate for inkjet computer-to-plate according to claim 7, **characterized in that** the alloy base is an alloy base of silica and aluminum, in which a content of silica is 30∼60 wt%, or
an alloy base of aluminum and zinc, in which a content of the zinc is 1∼3 wt%, or
an alloy base of aluminum and iron, in which a content of the iron is 0.1∼1 wt%.

9. An inkjet printing method, comprising the following steps: imparting image-text information on the plate according to any of claim 1 and claims 3-8 by using plate-making ink, cross-linking the plate-making ink and printing the plate having the image-text information, so as to obtain a presswork.

10. The inkjet printing method according to claim 9, **characterized in that** the plate-making ink is a solvent-based plate-making ink, which comprises:
| | |
|---|---|
| film forming resin | 1∼35 wt% |
| curing agent | 0.01∼5 wt% |
| nano-scale or micron-scale dyestuff | 0.01∼10 wt% |
| solvent | balance amount |
the film forming resin is at least one selected from the group consisting of polyacrylic acid resin, polymethacrylic acid resin, ester of polyacrylic acid resin, ester of polymethacylic acid resin, polyimide resin, methyl silicone resin, polyester resin, epoxy resin, phenolic resin, polyurethane resin, benzoxazine resin, alkyd resin, rubber, polyamide, polyvinyl chloride, polystyrene, polycarbonate, polyphenyl ether and polysulfone;
the curing agent is at least one selected from the group consisting of silicone oil, epoxy resin with a low molecular weight, dicyandiamide, melamine, ethanolamine, triethylamine, polyisocyanate, benzoyl peroxide, acetic anhydride, 2-ethylimidazole, 2,4-dimethyl imidazole, mellophanic dianhydride and N,N-dimethylaniline;
the nano-scale or micron-scale dyestuff has a particle size of 10∼3000 nm.

11. The inkjet printing method according to claim 10, **characterized in that** the ester of polyacrylic acid resin comprises a product of esterification reaction between the polyacrylic acid resin and C1∼C5 monobasic alcohols; the ester of the polymethacylic acid resin comprises a product of esterification reaction between the polymethacrylic acid resin and C1∼C5 monobasic alcohols;
the epoxy resin with a low molecular weight has an epoxy equivalent value of 100∼2000 g/equivalent.

12. The inkjet printing method according to claim 10, **characterized in that** the dyestuff in the plate-making ink is one selected from acidic dyestuff, active dyestuff or alkaline dyestuff.

13. The inkjet printing method according to claim 12, **characterized in that** the acidic dyestuff is one of dye acid blue 9, dye acid blue 9 SF and dye acid yellow 23 SF;
the active dyestuff is one of black dyestuff SP series or reactive black;
the alkaline dyestuff is one of basic brilliant blue and N,N-dimethylaniline in blue dyestuffs.

14. The inkjet printing method according to claim 10, **characterized in that** the solvent in the plate-making ink is one selected from ethylene glycol monomethyl ether, ethylene glycol monoethyl ether, ethylene glycol mono-*n*-butyl ether, ethylene glycol dimethyl ether, propylene glycol monomethyl ether, propylene glycol monoethyl ether, propylene glycol monomethyl ether acetate, propylene glycol monoethyl ether acetate, propylene glycol monobutyl ether acetate, ethylene glycol monobutyl ether acetate, N,N-dimethylformamide, dioxane, *sec*-butyl acetate, A grade mineral essential oil and B grade mineral essential oil.

## Patentansprüche

1. Platte für digitale Tintenstrahldruckplattenbelichtung, umfassend eine metallische Basis, eine Haftstoffschicht, die auf der Oberfläche der metallischen Basis beschichtet ist, und eine Tintenabstoßschicht, die auf der Haftstoffschicht beschichtet ist, wobei die Haftstoffschicht erhalten wird durch Beschichten und Trocknen eines Haftstoffsols, wobei das Haftstoffsol zur Beschichtung aus gelöstem Stoff und Lösungsmittel besteht, und wobei
die metallische Basis keinen Behandlungen eines elektrolytischen Körnens und Anodisierens ausgesetzt ist,
der Haftstoff in der Haftstoffschicht wenigstens einer ausgewählt aus der Gruppe bestehend aus Epoxyharz, Polyurethan, Polyolefin, Polyester, StyrolButadien-Kautschuk, Gelatine, Polyvinylbutyral, Polyamid, Kolophoniumharz, Polyvinylalkohol, Alkydharz und Polyvinylacetat ist,
die Tintenabstoßschicht Fluor-enthaltendes Harz ist.

2. Platte für digitale Tintenstrahldruckplattenbelichtung nach Anspruch 1, **dadurch gekennzeichnet, dass** die Tintenabstoßschicht mit einer Schutzschicht abgedeckt ist, welche ein Polymerfilm mit einer Dicke von 1∼20 µm ist,
wobei das Polymer in dem Polymerfilm wenigstens eines von Polyethylen, Polypropylen, Polypenten, Polyvinylalkohol, Polyvinylbutyral, Polystyrol, Polyethylenterephthalat, Polyvinylchlorid und Poly(vinylidendichlorid) ist.

3. Platte für digitale Tintenstrahldruckplattenbelichtung nach Anspruch 1, **dadurch gekennzeichnet, dass** die Konzentration des gelösten Stoffs in dem Haftstoffsol 0,05∼15 Gew.-% ist und die Beschichtungsmenge des Haftstoffsols 0,001∼10 g/m² ist, wobei der gelöste Stoff Haftstoff in dem Haftstoffsol ist; und/oder
die Tintenabstoßschicht durch Beschichten einer gemischten Flüssigkeit aus Fluor-enthaltendem Harz und organischem Lösungsmittel und Trocknen erhalten wird, wobei der Gehalt des Fluor-enthaltenden Harzes in der gemischten Flüssigkeit aus Fluor-enthaltendem Harz und organischem Lösungsmittel 0,01∼20 Gew.-% ist und die Beschichtungsmenge der gemischten Flüssigkeit aus Fluor-enthaltendem Harz und organischem Lösungsmittel 0,001∼5 g/m² ist.

4. Platte für digitale Tintenstrahldruckplattenbelichtung nach Anspruch 1 oder 3, **dadurch gekennzeichnet, dass** das Polyolefin wenigstens eines ausgewählt aus der Gruppe bestehend aus Polypropylen, Polyvinylchlorid und Polystyrol ist;
das Fluor-enthaltende Harz wenigstens eines aus Fluor-enthaltendem Acrylharz, Fluor-enthaltendem Isocyanatharz, Fluor-enthaltendem Expoxyharz und Fluor-enthaltendem Polyolefinharz ist;
das organische Lösungsmittel wenigstens eines ausgewählt aus der Gruppe bestehend aus Dimethylsulfoxid, Xylol, Butylacetat, Ethylenglycol, Propandiol, Butanol, Aceton und Chloroform ist.

5. Platte für digitale Tintenstrahldruckplattenbelichtung nach Anspruch 3, **dadurch gekennzeichnet, dass** das Lösungsmittel wenigstens eines ausgewählt aus der Gruppe bestehend aus Wasser, Ethanol, Ester von Disäure, Cyclohexan, Heptan, Tetrahydrofuran und aromatischem Lösungsmittel ist.

6. Platte für digitale Tintenstrahldruckplattenbelichtung nach Anspruch 5, **dadurch gekennzeichnet, dass** das aromatische Lösungsmittel wenigstens eines ausgewählt aus der Gruppe bestehend aus Benzylalkohol, Phenethylalkohol, Xylol, Ethylbenzol und Toluol ist.

7. Platte für digitale Tintenstrahldruckplattenbelichtung nach Anspruch 1, **dadurch gekennzeichnet, dass** die Metallbasis Aluminiumbasis oder Legierungsbasis ist.

8. Platte für digitale Tintenstrahldruckplattenbelichtung nach Anspruch 7, **dadurch gekennzeichnet, dass** die Legierungsbasis eine Legierungsbasis aus Siliziumdioxid und Aluminium ist, bei der ein Gehalt an Siliziumdioxid 30∼60 Gew.-% ist, oder
eine Legierungsbasis aus Aluminium und Zink, bei der ein Gehalt des Zinks 1∼3 Gew.-% ist, oder
eine Legierungsbasis aus Aluminium und Eisen, bei der ein Gehalt des Eisens 0,1∼1 Gew.-% ist.

9. Tintenstrahldruckverfahren, welches die folgenden Schritte umfasst: Vermitteln von Bild-Text-Information auf der Platte nach einem der Ansprüche 1 und Ansprüche 3 bis 8 durch Verwendung einer Platte-bildenden Tinte, Vernetzen der Platte-bildenden Tinte und Drucken der Platte mit der Bild-Text-Information, um eine Druckware zu erhalten.

10. Tintenstrahldruckverfahren nach Anspruch 9, **dadurch gekennzeichnet, dass** die Platte-bildende Tinte eine Platte-bildende Tinte auf Lösungsmittelbasis ist, welche umfasst:
| | |
|---|---|
| filmbildendes Harz | 1∼35 Gew.-% |
| | |
| Härtungsmittel | 0,01∼5 Gew.-% |
| | |
| Farbstoff im Nano-Maßstab oder Mikro-Maßstab | 0,01∼10 Gew.-% |
| | |
| Lösungsmittel | restliche Menge, |
wobei das filmbildende Harz wenigstens eines ausgewählt aus der Gruppe bestehend aus Polyacrylsäureharz, Polymethacrylsäureharz, Ester von Polyacrylsäureharz, Ester von Polymethacrylsäureharz, Polyimidharz, Methylsilikonharz, Polyesterharz, Epoxyharz, Phenolharz, Polyurethanharz, Benzoxazinharz, Alkydharz, Kautschuk, Polyamid, Polyvinylchlorid, Polystyrol, Polycarbonat, Polyphenylether und Polysulfon ist;
das Härtungsmittel wenigstens eines ausgewählt aus der Gruppe bestehend aus Silikonöl, Epoxyharz mit einem niedrigen Molekulargewicht, Dicyandiamid, Melamin, Ethanolamin, Triethylamin, Polyisocyanat, Benzoylperoxid, Essigsäureanhydrid, 2-Ethylimidazol, 2,4-Dimethylimidazol, Mellophansäuredianhydrid und N,N-Dimethylanilin ist;
der Farbstoff im Nano-Maßstab oder Mikrometer-Maßstab eine Teilchengröße von 10∼3000 nm aufweist.

11. Tintenstrahldruckverfahren nach Anspruch 10, **dadurch gekennzeichnet, dass** der Ester von Polyacrylsäureharz ein Produkt einer Veresterungsreaktion zwischen dem Polyacrylsäureharz und einwertigen C1∼C5-Alkoholen umfasst; der Ester des Polymethacrylsäureharzes ein Produkt einer Veresterungsreaktion zwischen dem Polymethacrylsäureharz und einwertigen C1∼C5-Alkoholen umfasst;
das Epoxyharz mit einem niedrigen Molekulargewicht einen Epoxyäquivalenzwert von 100∼2000 g/Äquivalent aufweist.

12. Tintenstrahldruckverfahren nach Anspruch 10, **dadurch gekennzeichnet, dass** der Farbstoff in der Platte-bildenden Tinte einer ist, der ausgewählt ist aus saurem Farbstoff, aktivem Farbstoff oder alkalischem Farbstoff.

13. Tintenstrahldruckverfahren nach Anspruch 12, **dadurch gekennzeichnet, dass** der saure Farbstoff einer von Farbstoff Säureblau 9, Farbstoff Säureblau 9 SF und Farbstoff Säuregelb 23 SF ist;
der aktive Farbstoff einer von schwarzem Farbstoff der SP-Reihe oder Reaktivschwarz ist;
der alkalische Farbstoff einer von basischem Brilliantblau und N,N-Dimethylanilin in blauen Farbstoffen ist.

14. Tintenstrahldruckverfahren nach Anspruch 10, **dadurch gekennzeichnet, dass** das Lösungsmittel in der Platte-bildenden Tinte eines ist, das ausgewählt ist aus Ethylenglycolmonomethylether, Ethylenglycolmonoethylether, Ethylenglycolmono-n-butylether, Ethylenglycoldimethylether, Propylenglycolmonomethylether, Propylen-glycolmonoethylether, Propylenglycolmonomethyletheracetat, Propylenglycol-monoethyletheracetat, Propylenglycolmonobutyletheracetat, Ethylenglycol-monobutyletheracetat, N,N-Dimethylformamid, Dioxan, sec-Butylacetat, essentiellen Mineralölen der Qualität A und essentiellen Mineralölen der Qualität B.

## Revendications

1. Plaque pour impression directe des plaques par jet d'encre, comprenant une base métallique, une couche d'adhésif qui couvre la surface de la base métallique et une couche repoussant l'encre qui couvre la couche d'adhésif, dans laquelle la couche d'adhésif est obtenue en couvrant et en faisant sécher un sol adhésif, dans laquelle le sol adhésif destiné au revêtement consiste en un soluté et un solvant et dans laquelle la base métallique n'est pas soumise aux traitements de grainage et d'anodisation électrolytiques,
l'adhésif de la couche d'adhésif est au moins l'un sélectionné dans le groupe consistant en une résine époxy, un polyuréthane, une polyoléfine, un polyester, un caoutchouc butadiène-styrène, une gélatine, un polybutyral vinylique, un polyamide, une résine de colophane, un alcool polyvinylique, une résine alkyde, et un polyacétate de vinyle,
la couche repoussant l'encre est une résine contenant du fluor.

2. Plaque pour impression directe des plaques par jet d'encre selon la revendication 1, **caractérisée en ce que** la couche repoussant l'encre est recouverte d'une couche protectrice qui est un film polymère ayant une épaisseur comprise entre 1 et 20 µm,
le polymère dans le film polymère est au moins l'un parmi le polyéthylène, le polypropylène, le polypentène, l'alcool polyvinylique, le polybutyral vinylique, le polystyrène, le polyéthylène térephtalate, le polychlorure de vinyle et le dichlorure de polyvinylidène.

3. Plaque pour impression directe des plaques par jet d'encre selon la revendication 1, **caractérisée en ce que** la concentration de soluté dans le sol adhésif est comprise entre 0,05 et 15 % en poids et la quantité efficace de revêtement du sol adhésif est comprise entre 0,001 et 10 g/m², le soluté est adhésif dans le sol adhésif ; et/ou
la couche repoussant l'encre est obtenue par revêtement avec un liquide mixte d'une résine contenant du fluor et un solvant organique et par séchage, dans laquelle la teneur en résine contenant du fluor dans le liquide mixte résine contenant du fluor et solvant organique est comprise entre 0,01 et 20 % en poids et la quantité efficace de revêtement du liquide mixte résine contenant du fluor et solvant organique est comprise entre 0,001 et 5 g/m².

4. Plaque pour impression directe des plaques par jet d'encre selon la revendication 1 ou 3, **caractérisée en ce que** la polyoléfine est au moins l'une sélectionnée dans le groupe consistant en le polypropylène, le polychlorure de vinyle et le polystyrène ;
la résine contenant du fluor est au moins l'une parmi la résine acrylique contenant du fluor, la résine isocyanate contenant du fluor, la résine époxy contenant du fluor et la résine polyoléfinique contenant du fluor ;
le solvant organique est au moins l'un sélectionné dans le groupe consistant en le diméthylsulfoxide, le xylène, l'acétate de butyle, l'éthylène glycol, le propanediol, l'alcool butylique, l'acétone et le chloroforme.

5. Plaque pour impression directe des plaques par jet d'encre selon la revendication 3, **caractérisée en ce que** le solvant est au moins l'un sélectionné dans le group consistant en l'eau, l'éthanol, l'ester de diacide, le cyclohexane, l'heptane, le tétrahydrofuranne et un solvant aromatique.

6. Plaque pour impression directe des plaques par jet d'encre selon la revendication 5, **caractérisée en ce que** le solvant aromatique est au moins l'un sélectionné dans le groupe consistant en l'alcool benzylique, l'alcool phénéthylique, le xylène, l'éthylbenzène et le toluène.

7. Plaque pour impression directe des plaques par jet d'encre selon la revendication 1, **caractérisée en ce que** la base métallique est une base en aluminium ou une base en alliage.

8. Plaque pour impression directe des plaques par jet d'encre selon la revendication 7, **caractérisée en ce que** la base en alliage est une base en alliage de silice et d'aluminium, dans laquelle la teneur en silice est comprise entre 30 et 60 % en poids, ou
une base en alliage d'aluminium et de zinc, dans laquelle la teneur en zinc est comprise entre 1 et 3 % en poids, ou
une base en alliage d'aluminium et de fer, dans laquelle la teneur en fer est comprise entre 0,1 et 1 % en poids.

9. Procédé d'impression par jet d'encre comprenant les étapes suivantes : communication des informations image-texte à la plaque suivant l'une quelconque de la revendication 1 et des revendications 3 à 8, en utilisant une encre de clichage, en faisant réticuler l'encre de clichage et en imprimant la plaque ayant les informations image-texte, de manière à obtenir un travail d'impression.

10. Procédé d'impression par jet d'encre selon la revendication 9, **caractérisé en ce que** l'encre de clichage est une encre de clichage à base de solvant, qui comprend :
| | |
|---|---|
| une résine filmogène | de 1 à 35 % en poids |
| | |
| un agent durcisseur | de 0,01 à 5 % en poids |
| | |
| un colorant à l'échelle nanométrique ou à l'échelle micrométrique | de 0,01 à 10 % en poids |
| | |
| un solvant | quantité restante |
la résine filmogène est au moins l'une sélectionnée dans le groupe consistant en la résine d'acide polyacrylique, la résine d'acide polyméthacrylique, la résine d'ester de l'acide polyacrylique, la résine d'ester de l'acide polyméthacylique, la résine de polyimide, la résine de méthylsilicone, la résine de polyester, la résine époxy, la résine phénolique, la résine polyuréthanne, la résine de benzoxazine, la résine alkyde, le caoutchouc, le polyamide, le polychlorure de vinyle, le polystyrène, le polycarbonate, l'éther polyphénilique et le polysulfone ;
l'agent durcisseur est au moins l'un sélectionné dans le groupe consistant en l'huile de silicone, la résine époxy de faible poids moléculaire, le dicyandiamide, la mélamine, l'éthanolamine, la triéthylamine, le polyisocyanate, le peroxyde de benzoyle, l'anhydride acétique, le 2-éthylimidazole, le 2,4-diméthylimidazole, le dianhydride mellophanique et la N,N-diméthylaniline ;
le colorant à l'échelle nanométrique ou à l'échelle micrométrique ayant une taille de particule comprise entre 10 et 3000 nm.

11. Procédé d'impression par jet d'encre selon la revendication 10, **caractérisé en ce que** la résine d'ester de l'acide polyacrylique comprend un produit de réaction d'estérification entre la résine d'acide polyacrylique et les alcools monobasiques C1 à C5 ; la résine d'ester de l'acide polyméthacylique comprend un produit de réaction d'estérification entre la résine d'acide polyméthacrylique et les alcools monobasiques C1 à C5 ;
la résine époxy de faible poids moléculaire a une valeur d'équivalent époxy de 100 à 2000 g/équivalent.

12. Procédé d'impression par jet d'encre selon la revendication 10, **caractérisé en ce que** le colorant dans l'encre de clichage est l'un sélectionné parmi un colorant acide, un colorant actif ou un colorant alcalin.

13. Procédé d'impression par jet d'encre selon la revendication 12, **caractérisée en ce que** le colorant acide est l'un parmi le bleu acide colorant 9, le bleu acide colorant 9 SF et le jaune acide colorant 23 SF ;
le colorant actif est l'un des colorants noirs série SP ou noir réactif ;
le colorant alcalin est l'un parmi le bleu brillant basique et la N,N-diméthylaniline dans les colorants bleus.

14. Procédé d'impression par jet d'encre selon la revendication 10, **caractérisé en ce que** le solvant dans l'encre de clichage est l'un sélectionné parmi l'éther monométhylique d'éthylène glycol, l'éther monoéthylique d'éthylène glycol, l'éther mono-n-butylique d'éthylène glycol, l'éther diméthylique d'éthylène glycol, l'éther monométhylique de propylène glycol, l'éther monoéthylique de propylène glycol, l'acétate d'éther monométhylique de propylène glycol, l'acétate d'éther monoéthylique de propylène glycol, l'acétate d'éther monobutylique de propylène glycol, l'acétate d'éther monobutylique d'éthylène glycol, le N,N-diméthylformamide, le dioxyde de diéthylène, le sec-butyl acétate, l'huile essentielle minérale de grade A et l'huile essentielle minérale de grade B.
